

June 29, 1926.

**1,590,608**

E. TAYLOR

INSULATED ELECTRICAL CONDUCTOR AND THE LIKE

Original Filed March 11, 1920



Edwin Taylor Inventor

By his Attorneys  
Ward, Crosby & Smith

Patented June 29, 1926.

1,590,608

# UNITED STATES PATENT OFFICE.

EDWIN TAYLOR, OF BROOKLYN, NEW YORK, ASSIGNOR TO TAYLOR LABORATORIES, INC., OF NEW YORK, N. Y., A CORPORATION OF NEW YORK.

## INSULATED ELECTRICAL CONDUCTOR AND THE LIKE.

Original application filed March 11, 1920, Serial No. 364,980. Divided and application filed June 17, 1924, Serial No. 720,520. Divided and this application filed March 18, 1926. Serial No. 95,802.

My invention relates to improvements in insulated electrical conductors and the like. The main object of the invention is to provide an electrical conductor with an improved insulation of organic material. The invention, however, may also be used for coating other objects than electrical conductors, for example ribbons, sheets, etc. of various materials. This application is a division of my prior application Ser. No. 720,520 filed June 17, 1924 which in turn is a division of my prior application Ser. No. 364,980 filed March 11, 1920.

Further and more specific objects, features and advantages will more clearly appear from the detail description given below taken in connection with the accompanying drawing which forms a part of the specification.

20 The drawing, partly in vertical section, illustrates more or less diagrammatically an apparatus adapted to put the main features of the improvements in one form.

According to my invention in its preferred form, I insulate or coat the conductor or other body with a layer of cellulose. I preferably do this by making a suitable solution of cellulose, applying a layer of this to the wire conductor or other body and removing

30 the solvent constituents from cellulose, leaving a homogeneous integrally continuous layer of cellulose on the body. I preferably remove the solvent constituents by electrolytic action. For this purpose I preferably

35 dissolve the organic material such as cellulosic material in a solution of zinc chloride or a solution of hydrated cupric oxide in concentrated ammonia. By such solution of the cellulose in zinc chloride or the cupro-

40 ammonia the cellulose is converted from the cellular or fibrous condition to a colloidal state. I preferably use a solution which is relatively concentrated and thick, and apply a suitable layer thereof to the body to be

45 coated and then subject the cellulose solution on the body to electrolysis whereby the cellulose is deposited more solidly upon the body to be coated which may serve as the anode, and the copper or zinc as the case may be, is

50 deposited on a cathode, the chlorine or ammonia being given off in gaseous form. Both the gas so given off, as well as the metal deposited on the cathode, may be recovered for re-use.

Referring to the drawing which illustrates an apparatus adapted for use in coating or covering rods or filaments of cellulose as well as metallic rods, wires and other objects, 10 represents a tank holding a solution of cellulose, 8 a pipe connection for supplying additional cellulose solution under pressure, and 9 a pipe for maintaining a gas pressure on the contents of tank 10. Through the side wall of 10 and near the bottom extends a nozzle 12 provided with a definite sized orifice 4, fitted with a perforated guide piece 44, as near the orifice 4 as the choke of the nozzle will permit. Projecting through the opposite wall of the tank 10 is a hollow fitting or nozzle 43, provided with a bore substantially the size of the object to be coated and placed central with the bore of nozzle 12. The nozzle 12 projects through the wall of a second tank 20, of any desired length, and fitted at its further wall with a stuffing box 75 having a central perforation 47, approximately of the diameter of the coated rod or wire. A vent pipe 33 is placed at the top of tank 20, for the removal by suction of gases released or generated during operation. 80

Below the level of the liquid in tank 20, and central with nozzle 12 and stuffing box 47, is suspended a tubular electrode 37 split lengthwise to facilitate removal, and provided with electric connections 38, the tube 85 being a cathode while in use. Beyond tank 20 and communicating with it by the stuffing box 47, is a third tank 50 containing a roller 48 at its further end.

The object to be coated, for instance a wire 46 on a reel 45, is led through nozzles 43 and 12, through guide piece 44, orifice 4, electrode 37, stuffing box 47, under roller 48, and to a reel 51, situated outside of tank 50 and so driven that it may place the wire 95 under enough tension to draw it from the reel and through the apparatus. Tank 10 is now filled with a viscous, concentrated solution of organic material such as cotton or silk dissolved for example in cupro-ammonia, or in the case of silk in nickel-ammonia alone or in a mixture of both cupro- and nickel-ammonia. Tank 20 is filled with a dilute acid solution and tank 50 with clean water. The reel 51 is now started drawing 100 the wire through the apparatus, pressure is applied to tank 10, through pipe 9 causing the cellulose to flow through orifice 4 and

an electric current is passed through the wire 46 by means of a contact shoe 28, and a conductor 29, connected to the positive pole of a source of electricity. The wire 46 while 5 passing through the tubular electrode 37, becomes an anode and 37 a cathode. The cellulose issuing between the wall of the orifice 4 and the centrally located wire 46 is caused to flow at a slower speed than the 10 wire and is drawn or stretched thereon in a uniform coating of any desired thickness the flotation effect of the bath materially preventing flow of the viscous solution after leaving nozzle 12 and before the cellulose 15 has been finally deposited on wire 46 by means of the current passing during the travel of the coated wire through the cathode 37 which is made long enough and the speed of the wire slow enough, to ensure the 20 removal and deposition of the metallic constituent and the release of the gaseous or volatile constituent. After passage through cathode 37 the wire now covered with a rubbery coating of deposited organic material 25 passes through the stuffing box 47 filling the bore thereof and so preventing the water in tank 50 from mixing with the acid liquid in 20 or vice-versa. The coated wire 49 is now well washed during passage through 30 tank 50 passes under under guide-roll 48, and to reel 51, it now being ready for drying or for further desired operations. It is obvious that in place of one wire or rod passing through orifice 4, any number of 35 wires may be passed in parallel each being separated from its neighbor by coating of cellulose, etc., and the whole enclosed in a like coating of any desired thickness. Furthermore the nozzles and apparatus may be 40 so constructed and placed that a twisted or cable effect may be imparted to the wires during coating.

The above process after drying, etc., results in a tough, elastic, transparent coating 45 which is substantially impermeable to oil and of any thickness or color, etc., desired, firmly adherent to the wire and of a high di-electric strength. The coating resulting from the above described process is substantially pure cellulose and the cellulose is 50 practically uncombined, that is, it is not combined with esters or other radicals to form compounds such as xanthates, nitrates, and the like. Successive coats of the same 55 or different material may be given by passing the covered wire as it leaves tank 50 through successive apparatus of the same kind, the coated wire still wet passing in at a nozzle similar to 43 but of larger bore to 60 accommodate the increased diameter.

In the application of this process and its modifications as applied to silk advantage 65 may be taken of the fact that silk will dissolve in nickel ammonia solution, while cotton will not, although cupro-ammonia dis-

solves both. Mixed silk and cotton waste goods, etc., may be separated and rendered of increased commercial value by first treating the mixed material with nickel-ammonia whereby the silk is dissolved and removed 70 from the cotton by filtration. The cotton may now be dissolved in cupro-ammonia and the silk and cotton solutions either singly or mixed in definite proportions, utilized for coating as above described, with a coating of silk or cellulose or a mixture thereof. The coatings may be dyed or colored as readily as the natural fiber and the mechanical strength of the deposited layer is but little less than that of the natural fiber. 75

As to the process in general the utmost care should be exercised to avoid all dust and dirt. The solutions must be carefully filtered and dirt kept out afterward. All the apparatus should be closed in wherever possible. The water employed for making up the solutions should be distilled or at any rate contain a minimum of mineral salts and should be free from carbonic acid gas if a fine filament or a perfectly transparent 90 product is desired.

The strength of the acid water must also be kept within reasonable limits although this is easy on account of the large volume in the tank compared to the amount circulated, changes in concentration taking place slowly. This acid water should also be kept free from grosser impurities and from CO<sub>2</sub>. 95

I prefer to use nitric acid as its ultimate product under electrolysis is always ammonia. The bath may be kept to strength by the simple addition of nitric acid, the ammonia released from the organic solution or formed by electrolysis being readily drawn from the top of the tanks and directly recovered, and any residual acid easily removed from the cellulose, etc., by washing.

Definite figures on the electrical current employed are also difficult to give on account of the many variations of the general process. A direct current is preferable; a pulsating current in one direction gives good results but takes a longer time. The problem is an electro-chemical one and the rate of deposition of both cellulose and metal is a function of the amperage rather than of voltage. For instance, in the electrolysis of cellulose dissolved in cupro-ammonia, I have used currents of 110 volts and a current density of  $\frac{1}{2}$  amp. per sq. inch of anode surface, while almost the same result may be obtained with 1.8 volts and  $\frac{100}{100}$  of an amp. per sq. inch, although the time required is longer. In general, only enough 110

amperage should be carried to secure a reasonably adherent deposit on the cathode, of the metallic solution constituent employed. If the current rate is unduly raised, 115 a spongy deposit of metal forms which is 120

125

apt to fall into the bath, adhere to the material being treated and otherwise cause trouble, while at the same time the bath overheats and more current passes than is required. Contrary to this a heavy amperage favors the deposition of cellulose. For cathodes a metal similar to the one used in the solvent, copper, nickel, zinc, etc., should be employed. With a little attention to the amperage passed all these metals may be deposited in a somewhat spongy condition and while adhering well to the cathode, may be easily scraped therefrom in a condition to be readily re-dissolved for the preparation of new solutions.

For dissolving the organic material, cellulose, silk, etc., if the solution is to be an ammoniacal one, I prefer to saturate 30% ammonia water, free from carbonate of ammonia, etc., with hydrated cupric or nickel oxides. The solutions are filtered through fibrous, nitro-cellulose, cooled to about 40° F. and saturated with the material to be dissolved in suitable mixing machines. The amount of material dissolved depends largely upon the fibre, etc., used varying somewhat with each different quality or grade of the same kind of material. Some raw cottons for instance will completely dissolve in the proportion of 1 lb. cotton to 20 lbs. of cupra, while with other varieties, 1 lb. cotton to 35 lbs. solution is the best that can be done. When using zinc chloride, I employ a saturated solution of the C. P. salt in distilled water, these solutions being even more sensitive to impurities than the ammonia ones and more difficult to handle and recover.

After solution is complete the viscous mass is allowed to stand for about 24 hours, during which time it becomes much more fluid and may be forced through a filter by means of pressure. A fine sand bed on top of a layer of nitro-cotton, which in turn is supported by a fine wire screen is quite satisfactory. When desired the solutions are now concentrated by centrifugal action.

At this stage other ingredients may be added to the more or less fluid solution. For instance, if a saturated solution of cotton, or

other cellulose in cupro-ammonia is employed it is evident that if more cellulose, say in a fibrous but rather finely divided state be added, this latter addition will be practically unaffected by the solution but it will increase the viscosity of the mass, necessitate a higher pressure to force it through the nozzles or dies and will materially reduce the shrinkage or drying, the result being a material of practically the same chemical composition throughout, part of which is in the fibrous or cellular condition and part of which has been solidified from a colloidal condition.

The final layer of organic material with which the body or wire is coated, is substantially non-fibrous and non-cellular in structure, and is substantially homogeneous and continuous.

While I have described my improvements in great detail and with respect to preferred embodiments thereof, I do not desire to be limited to such details and forms, since many changes and modifications may be made and the improvements embodied in widely different forms without departing from the spirit and scope thereof in their broader aspects; hence I desire to cover all forms coming within the language or scope of any one or more of the appended claims.

What I claim as new and desire to secure by Letters Patent, is:

1. An insulated electrical conductor comprising a conducting wire with an insulating coating of substantially non-fibrous, structureless and uncombined cellulose thereon, said coating being substantially transparent, homogeneous and substantially continuous throughout and substantially impermeable to oil.

2. A body having thereon a coating of substantially pure cellulose, the cellulose being substantially noncellular and structureless and uncombined and forming a substantially continuous coating substantially impermeable to oil.

In testimony whereof I have signed my name to this specification.

EDWIN TAYLOR.